

(No Model.)

J. MAKIN.

LEAD LINED BOILER FOR PAPER PULP.

No. 344,120.

Patented June 22, 1886.

Fig. 1.



Fig. 2.



Witnesses.

John F. C. Prindler  
Fred L. Emery

Inventor.

J. Makin  
by Crosby & Gregor Allis

# UNITED STATES PATENT OFFICE.

JOHN MAKIN, OF BELFIELD; NEAR ROCHDALE, COUNTY OF LANCASTER, ENGLAND, ASSIGNOR TO CHARLES C. SPRINGER, TRUSTEE, OF YARMOUTH, MAINE.

## LEAD-LINED BOILER FOR PAPER-PULP.

SPECIFICATION forming part of Letters Patent No. 344,120, dated June 22, 1886.

Application filed April 27, 1886. Serial No. 200,312. (No model.)

*To all whom it may concern:*

Be it known that I, JOHN MAKIN, of Bel-  
field, near Rochdale, in the county of Lancas-  
ter, England, manager of a paper-works, have  
5 invented an Improvement in Lead-Lined Boil-  
ers for Paper-Pulp, of which the following de-  
scription, in connection with the accompa-  
nying drawings, is a specification, like letters on  
the drawings representing like parts.

10 In the manufacture of paper-pulp from wood  
by the so-called "sulphite process" it is nec-  
essary to provide the boiler with a lining,  
coated or covered at its inner side with lead  
or other usual acid-resisting metal.  
15 Patent of the United States No. 335,943,  
dated February 9, 1886, shows and describes  
a compound lining consisting of a foundation-  
plate, preferably of iron, covered on both sides  
with lead, the lead being caused to adhere to  
20 the foundation-plate by casting.

In practice it has been found that sheet-lead  
forms the most serviceable face; but great dif-  
ficulty has been experienced in securing the  
sheet-lead to the foundation-plate.

25 In my experiments to employ sheet-lead I  
have discovered that the same may be firmly  
secured or anchored to the foundation-plate by  
means of solder dropped into the holes made  
in the plate, the said solder attaching itself to  
30 the lead opposite the said holes, the said lead  
being partially melted opposite the holes be-  
fore the introduction of the solder.

35 My invention therefore consists in a novel  
method of attaching sheet-lead to a founda-  
tion-plate in the manufacture of a compound  
lining for pulp-forming boilers.

My invention consists, essentially, in plac-  
ing the foundation-plate and sheet-lead in con-  
tact, then partially fusing the lead opposite  
40 the holes in the foundation-plate, and running  
molten solder into the said holes to unite them  
with the partially-fused portion of the sheet-  
lead, the said solder filling the said holes and  
attaching itself firmly to the sheet-lead, con-  
45 stituting a series of bolts or anchors to hold  
the sheet-lead in place on the foundation-plate  
and prevent it from creeping. The term  
"creeping" is fully explained in said patent.

Figure 1 represents a piece of lead lining

suitable to be applied to a boiler, shell, or tank 50  
for the production of wood or other fibrous  
pulp by a process wherein acid is employed;  
and Fig. 2 is a section of Fig. 1 in the dotted  
line *x* *x*, the said figure also showing a small  
portion of the boiler.

55 The boiler or other vessel *a*, a portion of  
which is shown in Fig. 2, is or may be of any  
usual shape commonly employed in the manu-  
facture of wood pulp.

The compound lining is composed, essen- 60  
tially, of a foundation-plate, *b*, having a series  
of holes, *b'*, and preferably the entire surface  
of the foundation-plate will be covered with  
tin or zinc by a dipping or galvanizing pro- 65  
cess, in order that the lead or solder brought  
in contact therewith may more readily adhere  
thereto.

In the drawings I have represented the tin-  
ning or galvanizing by the letter *g*; but the  
thickness of the tinning or galvanizing is ex- 70  
aggerated.

The sheet-lead, *l*, to be used will in practice  
be about three-eighths of an inch thick, more  
or less. The foundation-plate, preferably  
75 tinned or galvanized, will be laid upon the  
sheet-lead *l*.

As herein shown, it is supposed that the com-  
pound lining is to have a straight side; but  
the compound lining may be made to present  
any curve by first bending the foundation-plate 80  
to the proper curve and by employing a tem-  
plate of the proper curve, upon which the sheet-  
lead will be laid, the curved foundation-plate  
being thereafter laid upon the sheet-lead.

Assuming that the foundation-plate and 85  
sheet-lead have been placed in contact, the op-  
erator by means of a blow-pipe will blow the  
flame into the holes *b'* and partially melt that  
part of the sheet-lead opposite the lower end  
90 of the holes, and while the same is yet in  
molten state will fill the said hole with molten  
solder, which will combine with the molten  
lead, constituting, as it were, a solder rivet  
integral with the lead lining.

Sheet-lead *l*, anchored, as described, at fre- 95  
quent intervals by means of solder, bolts, or  
rivets *d*, will be found to be so firmly attached  
to the foundation-plate that the lead will not

creep on or detach itself from the foundation plate.

Herein I have not considered it necessary to show the entire pulp-boiler; but the same may 5 and preferably will be spherical, or of the shape represented in the said Makin patent.

The edges of the compound lining will be united together in any usual manner—as, for instance, in the said patent or in United States 10 Patent No. 335,046.

By the term "solder" I mean any usual fusible solder mixture.

I claim—

An improvement in the art or method of 15 manufacturing compound linings for boilers, which consists in placing the sheet-lead and

perforated foundation-plate together, partially fusing the lead opposite the holes in the foundation-plate, and filling in the said holes with solder, the solder attaching itself to the sheet-lead and holding the same in place upon the foundation-plate, substantially as described. 20

In testimony whereof I have signed my name to this specification in the presence of two subscribing witnesses.

JOHN MAKIN.

Witnesses:

ALFRED GRUNDY,  
104 King Street, Manchester, England, Solicitor.

W.M. T. JONES,  
104 King Street, Manchester, England, Solicitor's  
Clerk.